

## UNITED STATES PATENT OFFICE

2,662,831

## METHOD OF BONDING COPPER TO ALUMINUM OR ALUMINUM ALLOYS

Carl R. Culverhouse, Jr., Birmingham, Ala., assignor to Anderson Brass Works, a corporation of Alabama

No Drawing. Application July 19, 1950,  
Serial No. 174,796

10 Claims. (Cl. 117—50)

1

This invention relates to a chemically coated aluminum article and the method of producing the same, and has for its principal object the provision of such a method whereby a suitable metal is chemically deposited on the aluminum from an alkali bath and is then chemically replaced by another metal from an acid bath containing complex ions, said replacing metal being below the metal replaced in the activity series of metals, thus obtaining as a result an aluminum article having directly, strongly adherently bonded to its surface a coating of the desired metal.

Another object of my invention is to provide a method of coating aluminum with copper whereby zinc is first chemically deposited on the aluminum from an alkali bath and is then replaced by copper by chemical reaction from an acid bath of copper fluoborate.

A further object is to provide a method of coating articles of both pure aluminum and aluminum alloys whereby a strongly adherent and even coating is deposited on the same and in which the adherability of the coating is substantially unaffected by the particular kind of aluminum alloy to be coated.

A further object is to provide a method of electroplating aluminum whereby it is unnecessary to first provide a cyanide strike or coating before electroplating, resulting in a direct bond between the base metal and the coating.

Briefly, my invention comprises degreasing and chemically cleaning the article of aluminum or aluminum alloy to be coated. The article thus cleaned is immersed in a sodium or potassium zincate solution where an even coating of zinc is obtained thereon. The zinc coated article is rinsed in water and then immersed in an acid solution of copper fluoborate where the zinc goes into solution and is chemically replaced on the surface of the article by the copper from the copper fluoborate solution.

Heretofore, so far as I am aware, coatings of copper have been deposited on pure aluminum and special processes have been devised to coat particular aluminum alloys, but there has been no satisfactory method of coating pure aluminum and all aluminum alloys with copper by any one process. I have found that by first coating aluminum or aluminum alloys with zinc and then chemically replacing the zinc with copper an even and strongly adherent coat of copper is obtained. I have thus provided a process equally adaptable to coating aluminum or aluminum alloys which is not dependent upon the

2

particular type of alloy to be coated, thereby making it possible to employ substantially the same process for coating pure aluminum or any of its alloys.

5 As stated, my invention is carried out by first degreasing the article of aluminum or aluminum alloy to be plated. This may be done by vapor degreasing with an organic solvent such as trichloroethylene, by immersion in an organic solvent such as carbon tetrachloride, or by washing the aluminum with a detergent or an emulsion cleaner. The degreased aluminum article is next chemically cleaned by first immersing it in a concentrated solution of nitric acid for approximately 30 seconds and then rinsing the article in water. Next, the article is immersed in 20 10% caustic soda for approximately 15 seconds thereby giving a light caustic etch to the surface of the aluminum and then rinsed in water. The time of caustic etching may vary with the alloy of aluminum to be coated. In any case, only a light caustic etch is necessary. The aluminum article is then immersed for 15 seconds in a solution consisting of 3 parts concentrated 15 nitric acid and 1 part 48% hydrofluoric acid and again rinsed in water.

15 The aluminum article thus chemically cleaned is coated with a uniform coating of zinc by immersing it for approximately 2 minutes in a solution of sodium zincate or potassium zincate having a pH at such a value that the aluminum will not be burned. I have found in actual practice that a pH of approximately 10 is satisfactory for most aluminum alloys. The zincate solution may 20 consist of approximately 100 grams per liter of zinc oxide and approximately 525 grams per liter of sodium hydroxide. While the zinc coating produced on the aluminum by this immersion is even and strongly adherent, an outer spongy coating of zinc is formed over the adherent coating of zinc which may be removed by rinsing the article in water.

25 After removing the outer spongy portion of the zinc coating, it is immersed in an acid solution which may consist of approximately 448 grams per liter of copper fluoborate (37.5° to 39° Baumé). The temperature of the copper fluoborate solution is maintained at from 80 to 170° F. while the zinc coated aluminum is immersed 30 therein. Any suitable vessel, such as one made from methyl methacrylate may be used for the acid bath. The zinc coating on the aluminum is chemically replaced by the copper from the copper fluoborate solution, the zinc ions going 35 into solution. A very thin and uniform coating

of copper is thus obtained on the aluminum. A complete coating of the copper for the aluminum is assured since the chemical reaction continues until the zinc is completely replaced by the copper. This thin coating of copper may be built up by methods of electroplating on copper which are well known in the art to which my invention relates. It will be apparent that metals other than copper may be electroplated on said copper coating.

From the foregoing it will be apparent that I have devised an improved method of coating aluminum and its alloys. I provide an even and strongly adherent coating of copper on the aluminum by chemically replacing a chemically deposited coating of zinc with the copper, and hence the coating does not blister or become separated from the surface of the aluminum. For use in those cases where pure aluminum and aluminum alloy articles are to be plated, my invention makes unnecessary the provision of separate vats and equipment, hence reducing equipment costs in the plating plant.

While I have described my invention in but one form, it will be obvious to those skilled in the art that it is not so limited, but is susceptible of various changes and modifications without departing from the spirit thereof, and I, desire, therefore, that only such limitations shall be placed thereupon as are specifically set forth in the appended claims.

What I claim is:

1. The method of firmly bonding a coating of copper directly to an aluminum article comprising degreasing the surface of the article, cleaning the surface of the article by immersing the same in a concentrated nitric acid solution and subsequently rinsing the article with water, immersing the article in an aqueous caustic soda solution and subsequently rinsing with water, immersing the article in an aqueous solution consisting of concentrated nitric acid and hydrofluoric acid and subsequently rinsing with water, depositing zinc on the article by immersing it in an aqueous solution of an alkali zincate having a controlled pH of approximately 10, rinsing the zinc-coated article with water, and chemically replacing the zinc with copper by immersing the zinc-coated article in an aqueous acid solution of copper fluoborate.

2. The method of firmly bonding a coating of copper directly to an aluminum article comprising degreasing the surface of the article, cleaning the surface of the article by immersing the same in a concentrated nitric acid solution for approximately 30 seconds and rinsing the article with water, immersing the aluminum article for approximately 15 seconds in an aqueous caustic soda solution and subsequently rinsing with water, immersing the article in an aqueous solution consisting of approximately 3 parts concentrated nitric acid and 1 part 48% hydrofluoric acid and subsequently rinsing with water, depositing zinc on the article by immersing it for approximately two minutes in an aqueous solution of sodium zincate having a controlled pH of approximately 10, rinsing the zinc-coated article with water, and chemically replacing the zinc with copper by immersing the zinc-coated article in an aqueous acid solution of copper fluoborate at a temperature of from 80° to 170° F.

3. The method of firmly bonding a coating of copper directly to an aluminum article as defined in claim 2 in which the zincate solution consists of approximately 100 grams per liter of zinc oxide and approximately 525 grams per liter of sodium hydroxide.

4. The method of firmly bonding a coating of copper directly to an aluminum article as defined in claim 2 in which the copper fluoborate solution consists of approximately 448 grams per liter of copper fluoborate at 37.5° to 39° Baumé.

5. The method of firmly bonding a coating of copper directly to an aluminum article as defined in claim 2 in which the article is degreased in trichloroethylene vapors.

6. The method of firmly bonding a coating of copper directly to an aluminum article as defined in claim 2 in which the article is degreased by immersion in a solution of carbon tetrachloride.

7. The method of firmly bonding a coating of copper directly to an aluminum article as defined in claim 2 in which the article is degreased with a detergent.

8. The method of firmly bonding a coating of copper directly to aluminum or aluminum alloys comprising degreasing and cleaning the surface of the aluminum to be coated, immersing the aluminum thus degreased and cleaned in an aqueous solution of potassium zincate, thereby depositing zinc on the aluminum, and chemically replacing the zinc with copper by immersing the zinc-coated aluminum in an aqueous acid solution of copper fluoborate.

9. The method of firmly bonding a coating of copper directly to aluminum or aluminum alloys comprising degreasing and cleaning the aluminum to be coated, immersing the aluminum thus degreased and cleaned in an aqueous solution of sodium zincate thereby depositing zinc on the aluminum, and chemically replacing the zinc with copper by immersing the zinc-coated aluminum in an aqueous acid solution of copper fluoborate.

10. The method of firmly bonding a coating of copper directly to aluminum or aluminum alloys comprising degreasing and cleaning the aluminum to be coated, immersing the aluminum thus degreased and cleaned in an aqueous solution of an alkali zincate, thereby depositing zinc on the aluminum, and chemically replacing the zinc with copper by immersing the zinc-coated aluminum in an aqueous acid solution of copper fluoborate.

CARL R. CULVERHOUSE, JR.

55 References Cited in the file of this patent  
UNITED STATES PATENTS

| Number    | Name         | Date          |
|-----------|--------------|---------------|
| 723,717   | Nicholson    | Mar. 24, 1903 |
| 1,405,534 | Merritt      | Feb. 7, 1922  |
| 1,457,149 | Cunningham   | May 29, 1923  |
| 1,627,900 | Hewitson     | May 10, 1927  |
| 2,398,738 | Gilbert      | Apr. 16, 1946 |
| 2,403,426 | Doutz et al. | July 2, 1946  |
| 2,580,773 | Heiman       | Jan. 1, 1952  |

OTHER REFERENCES

Struyk et al., Copper Plating from Fluoborate Solutions, Amer. Electroplater's Soc. vol. 33, September 1946, pages 923-934.